

June 16, 1942.

W. I. PATNODE

2,286,759

METHOD OF MAKING INSULATED WIRE OF SMALL OR IRREGULAR CROSS-SECTION

Filed Nov. 18, 1940

Fig. 2.



Fig. 1.



Fig. 3.



Fig. 5.



Fig. 4.



Fig. 6.



INSULATING COATINGS LABELED 2 COMPRIZE  
HEAT TREATED REACTION PRODUCT OF AN  
ALDEHYDE WITH A HYDROLYZED POLYMERIZED  
VINYL ESTER

Inventor:  
Winton I. Patnode,  
by Harry E. Junkin  
His Attorney.

## UNITED STATES PATENT OFFICE

2,286,759

METHOD OF MAKING INSULATED WIRE OF  
SMALL OR IRREGULAR CROSS-SECTIONWinton I. Patnode, Schenectady, N. Y., assignor  
to General Electric Company, a corporation of  
New York

Application November 18, 1940, Serial No. 366,176

1 Claim. (Cl. 91—70)

This invention relates to a method of making insulated wires of small or non-circular cross-section.

This application is a continuation in part of my copending application Serial No. 291,873, filed August 25, 1939, and assigned to the same assignee as the present invention.

Metallic conductors, such as magnet wires, have been insulated or coated with enamels or other resinous insulating materials by applying the coating material in a liquid state to the conductor and then baking the conductor to harden the insulation thereon. Magnet wires have also been insulated by extrusion of a hot, plastic resinous insulation thereon, which becomes hard upon cooling. Ordinarily, the magnet wires insulated or coated by either of these methods are of circular cross-section, and although wires of square or rectangular cross-section have been so insulated, the coating of wires of other than circular cross-section has always been kept to a minimum owing to two disadvantages in the processes. In the first place, coating a rectangular wire with an enamel or similar liquid composition by the conventional method of drawing the wire through a bath of the liquid composition and then baking the coating to harden it, results in a coating that is thick on the flat surfaces of the conductor and very thin on the edges or angular parts of the conductor. Consequently, in order adequately to insulate the edges or more angular parts of the conductor, it is necessary to apply much more material to the flat portion than is necessary or desirable. In the second place, the insulation of wires of rectangular cross-section by extrusion of the hot, plastic, resinous composition around the wire, as it is drawn through a rectangular die, is an uneconomic process, owing to the large number of different sizes of dies which are necessary. For example, the electrical industry uses at least a thousand different sizes of rectangular wires. They usually are insulated by wrappings of textiles or paper.

The insulation of very fine round wires, for example, less than 0.002 inch in diameter, is a difficult and expensive process owing to the fact that most liquid coating materials tend to form beads along the wire rather than to spread out in an even continuous coating, and also owing to the fact that the very low tensile strength and almost invisible size of such wires require very special machinery and technique.

The foregoing disadvantages of coating wires with thin films of resinous material have practically restricted the industry to the use of round

wires of greater than 0.002 inch in diameter and wires of less than this diameter or of non-circular cross-section are seldom insulated with a thin film of resinous material, in spite of the fact that there are great advantages to be attained through the use of such wires. For example, thin films of resinous insulation are generally superior to other types of magnet wire insulation, and rectangular wire effectively occupies less space when wound into a coil than does round wire of the same cross-sectional area.

No difficulty presents itself ordinarily in coating metallic conductors of average size circular cross-section by the conventional enameling process. It has, however, not been possible to reduce the diameter of the insulated wire once the enamel film is in place because the mechanical operations incident to such processes as rolling, drawing or swaging removed or destroyed the insulation film.

I have discovered that conductors insulated with polyvinyl acetal type materials, that is, resinous compositions comprising the reaction product of an aldehyde with a hydrolyzed polymerized vinyl ester, lend themselves to such mechanical treatment as above noted and can be reduced in size or shape without injury to the insulation film. Although it has been known that such coated wires can be deformed mechanically as by bending or hammering at any particular point without injury to the insulation at the point of deformation, it was not expected that such insulated wire could be continuously altered in cross-sectional size and shape, as by rolling, drawing or swaging, and despite such drastic mechanical treatment of the film, preserve its continuity which is essential in the production of insulated wire.

The advantages of this discovery will be readily apparent when it is realized that the process described herein overcomes the difficulties inherent in the previous methods of manufacturing conductors of comparatively small diameter or conductors of substantially non-circular cross-section provided with uniform resinous insulating coatings. As coating dies and the like are best adapted to the coating of circular wire, the present invention permits the use of the usual coating apparatus for applying the polyvinyl acetal resins to the wire which, after baking to harden the film, can be passed through ordinary rolls, such as turks head rolls, to produce flat or substantially rectangular wire, or drawn through the usual wire drawing dies to produce wire of small size or cross-section without impairing the

continuity of the insulating film. Furthermore, the herein-described process permits a substantial saving in cost, since wires of many different cross-sectional dimensions can be manufactured from one standard round insulated wire.

In accordance with this invention, a wire 0.032" in diameter coated with a 0.001" layer of the polyvinyl acetal resin enamel can be continuously cold rolled to a flat or substantially rectangular wire approximately 0.015" thick and 0.047" wide without breaking the insulating film. Again, a wire having a diameter of 0.0089" and an insulating coating 0.0008" thick can be rolled by passing the wire through suitable rolls until a flat wire 0.006" by 0.0141" was obtained. This wire, when tested for insulation breakdown by dipping the wire connected to one electric supply lead into a bath of mercury connected to the other supply lead, shows no breaks in the insulating film under ordinary voltage requirements whereas wires insulated with ordinary enamels will show numerous breaks in the enamel after being subjected to the rolling treatment. Since it effectively occupies less space when wound into a coil than round wire of the same cross-sectional area, the flat or rectangular wire so produced can be packed or wound closer than round wire so that in winding coils such as instrument coils and the like, more rectangular wire than round wire can be applied for equal coil volume or size.

A suitably coated 2 mil wire may be continuously drawn to one-quarter its original cross-section without impairing the insulation while a wire 18 mils in diameter coated with 1.0 mil layer of the enamel may be reduced by drawing to a diameter of 11.3 mils without breaking the enamel film. The extremely fine wire is particularly useful, in that instrument coils now may be wound from previously and uniformly 40 insulated wire of a size heretofore unattainable. Some increase in the length of the insulated conductor is noted with any of the above treatments. This increase may amount to approximately 20 per cent in certain instances.

In the accompanying drawing, Figure 1 illustrates one arrangement whereby a coated wire of circular cross-section may be converted into an insulated wire having a substantially rectangular cross-section, while Figure 4 shows an arrangement whereby a similarly coated wire may be reduced in cross-sectional area. The remaining Figures 2, 3, 5 and 6 are enlarged views of the insulated wire before and after being subjected to mechanical working. For example, a conductor 1 provided with the preferred baked organic enamel 2, originally having a circular cross-section as shown in Figure 2 will, after a suitable number of passes between rolls 3 and 4 as shown in Figure 1, assume a shape similar to that shown in Figure 3 which shape has been referred to as substantially rectangular. Like-

wise, an insulated wire such as shown in Figure 5 may have its cross-sectional area reduced as shown in Figure 6, by passing the wire through a wire drawing die such as the die shown in cross-section in Figure 4, in which a properly drilled diamond 5 is mounted in a support 6. It is to be understood that the shape or size of the insulated wire may be altered to even greater extent than indicated in the drawing.

The rolled conductor shown in Figure 3 or the drawn conductor of Figure 6 can be further worked to either a flatter or finer insulated conductor depending to some extent on the original size of the conductor and thickness of the baked insulating coating. When a considerable altering of the cross-sectional profile of the conductor is desired, it is usually best to obtain the desired result by a number of passes through progressively smaller dies or rolls. Further a rolled conductor, such as shown in Figure 3, may be made to assume a more rectangular shape by passing it through a pair of rolls similar to those shown in Figure 1 positioned at right angles to the rolls previously used. In every instance it is to be noted that some reduction in the thickness of the enamel coating takes place. The important feature is that, by these methods, it is possible to prepare extremely fine or substantially rectangular wire having practically uniform and wholly continuous insulation thereon, which wire is superior to that prepared by the usual methods previously attempted wherein a liquid coating material is applied to a very fine or non-circular conductor in its final shape.

As the cold working of the copper wire may harden it to a springy condition, which is a disadvantage in winding coils or for many other uses, it is desirable to anneal the coated wire to soften it after it has been cold worked. The anneal may be carried out by heating the springy wire in a high frequency electric field or in an oven held at 250°-300° C. Such treatment will not impair or otherwise alter the desirable properties of the enamel nor will the film be broken by subsequent winding operations. The time required for the anneal will depend on the wire used but will ordinarily be less than one minute.

What I claim as new and desire to secure by Letters Patent of the United States is:

The method of forming an insulated conductor having a closely-adhering, uniform coating thereon which comprises coating a conductor with a liquid coating composition comprising the reaction product of an aldehyde and a hydrolyzed polyvinyl ester, baking said coated conductor to harden the coating thereon, continuously drawing said coated conductor through a wire drawing die to alter the diameter thereof, and annealing said drawn conductor.

WINTON I. PATNODE.